

# UNITED STATES PATENT OFFICE.

JOHN T. H. DEMPSTER, OF SCHENECTADY, NEW YORK, ASSIGNOR TO GENERAL ELECTRIC COMPANY, A CORPORATION OF NEW YORK.

## ELECTRIC-RESISTANCE CONDUCTOR.

No. 901,428.

Specification of Letters Patent.

Patented Oct. 20, 1908.

Application filed November 4, 1907. Serial No. 400,691.

To all whom it may concern:

Be it known that I, JOHN T. H. DEMPSTER, a citizen of the United States, residing at Schenectady, county of Schenectady, State of New York, have invented certain new and useful Improvements in Electric-Resistance Conductors, of which the following is a specification.

This invention relates to the production of an alloy having certain valuable properties adapting it to a wide range of uses. It is heat refractory to an extraordinary degree and does not easily oxidize when subjected to a prolonged red heat in the atmosphere. It resists the action of moisture and is very acid proof, being insoluble in even concentrated mineral acids, boiling strong aqua regia being required for its solution. It has a high electrical resistivity, which adapts it well for electric heating and rheostat work since it withstands a red heat for a long continued service, and although under such conditions, it oxidizes slowly, the oxid is coherent and does not materially change its conductivity.

In the best composition I have thus far used, the alloy is composed approximately of

|    |                   |            |
|----|-------------------|------------|
| 62 | parts (by weight) | nickel,    |
| 20 | "                 | iron,      |
| 13 | "                 | chromium,  |
| 5  | "                 | manganese. |

The manganese is present in a sufficiently large proportion to lend its properties as a metal, the amount being more than sufficient to aid in the formation of the alloy.

An alloy containing

|        |                   |             |
|--------|-------------------|-------------|
| 62.040 | parts (by weight) | nickel,     |
| 20.164 | "                 | iron,       |
| 12.630 | "                 | chromium,   |
| 4.910  | "                 | manganese,  |
| .130   | "                 | silicon,    |
| .040   | "                 | carbon,     |
| .021   | "                 | phosphorus, |

produces a metal capable of being rolled and

drawn into extremely fine wire or ribbon having a resistivity of 117 microhms per cubic centimeter or 70 times that of pure copper. The alloy may be prepared in a powerful furnace, such as an oil furnace, and then worked in the ordinary way by rolling and drawing.

It will be understood, of course, that I do not limit my invention to the specific materials and proportions thereof herein set forth except in so far as it is limited by the scope of the claims annexed hereto.

What I claim as new and desire to secure by Letters Patent of the United States, is,—

1. An alloy containing iron, nickel, chromium and a manganese content exceeding 3%, the iron content not exceeding 50%.
2. An alloy containing iron, nickel, chromium, and a manganese content exceeding 3%, the nickel being in excess of the other ingredients.

3. An alloy containing iron, nickel, chromium, and a manganese content exceeding 3%, the iron and nickel being severally in excess of the other ingredients.

4. An alloy containing nickel, iron, chromium, and a manganese content of approximately 5%, the iron content not exceeding 50%.

5. An alloy containing nickel, iron, chromium, and a manganese content of approximately 5%, the nickel being in excess of the other ingredients.

6. An alloy containing nickel, chromium, and an iron content exceeding 10% and not exceeding 50%.

7. An alloy containing nickel, chromium, and an iron content of approximately 20%.

In witness whereof, I have hereunto set my hand this 2nd day of November, 1907.

JOHN T. H. DEMPSTER.

Witnesses:

BENJAMIN B. HULL,  
HELEN ORFORD.